# EUROPEAN PATENT SPECIFICATION

(11) **EP 1 558 701 B1**
(45) Date of publication and mention of the grant of the patent: **12.08.2009**
(21) Application number: 03810426.1
(22) Date of filing: 30.10.2003
(51) Int. Cl.: C10G 2/00

(54) **FISCHER-TROPSCH PROCESS USING A FISCHER-TROPSCH CATALYST AND A ZEOLITE-CONTAINING CATALYST**
FISCHER-TROPSCH-VERFAHREN, BEI DEM MAN EINEN FISCHER-TROPSCH-KATALYSATOR UND EINEN ZEOLITHHALTIGEN KATALYSATOR VERWENDET
PROCEDE FISCHER-TROPSCH FAISANT APPEL A UN CATALYSEUR FISCHER-TROPSCH ET A UN CATALYSEUR CONTENANT DES ZEOLITES

(30) Priority: 05.11.2002 EP 02079646; 19.11.2002 US 427408 P
(43) Date of publication of application: 03.08.2005
(73) Proprietor: Albemarle Netherlands B.V., 3818 LH Amersfoort (NL)
(72) Inventor: STEENWINKEL, Edgar, Evert, NL-2011 WD Haarlem (NL); SPEE, Marieke, Paulyne, Rénate, NL-3524 AS Utrecht (NL); VERLAAN, Johannes, Petrus, Jozef, 7415 DL Deventer (NL); VOGT, Eelco, Titus, Carel, 4105 DW Culemborg (NL)
(74) Representative: Rasser, Jacobus Cornelis
(86) International application number: PCT/EP2003/012166
(87) International publication number: WO 2004/041970

(56) References cited:
- US-A- 3 254 023
- US-A- 4 906 671
- US-A- 5 928 980

## Description

The present invention relates to a Fischer-Tropsch process for the conversion of carbon monoxide and hydrogen to C₅⁺ hydrocabon mixtures using a Fischer-Tropsch catalyst and a zeolite-containing catalyst.

The Fischer-Tropsch process generally comprises the following process steps. The first step involves reacting a source of carbon (such as coal or natural gas) with a source of oxygen (such as steam, air or oxygen) to form a mixture of carbon monoxide and hydrogen, usually referred to as synthesis gas.
The second step involves contacting the carbon monoxide and hydrogen with a Fischer-Tropsch catalyst leading to hydrocarbons and water. Depending on the process conditions and the catalyst used, the nature of the hydrocarbons and the chain length may vary. The main products of the Fischer-Tropsch reaction are linear olefins and paraffins and water, but limited isomerisation and inclusion of heteroatoms such as oxygen may occur. Generally applied catalysts for this second step are iron and/or cobalt-containing catalysts. In order to enhance isomerisation during this second step, a co-catalyst can be added.
The third step involves isomerisation of the hydrocarbons formed in the second step to produce more valuable products. For instance, the longer chains in the product may be cracked to form products in the diesel or gasoline range, and linear paraffins may be isomerized to improve diesel product properties like cloud point and pour point. Generally, adapted hydrotreating catalysts are used for this third step.

US 5,928,980 discloses the use - in the second step of the Fischer-Tropsch process - of a spent fluid catalytic cracking (FCC) catalyst impregnated with a group VIII metal, preferably cobalt and/or iron. This catalyst composition is prepared by impregnating the spent FCC catalyst with a metal salt, calcining the impregnated FCC catalyst to obtain a supported metal oxide, and reducing the metal oxide to the metal in a reducing gas atmosphere. The impregnated metal serves as the Fischer-Tropsch catalyst.

The preparation of this prior art catalyst composition requires a cumbersome process - involving the steps of impregnation, calcination, and reduction. It is therefore an object of the present invention to provide a process for the conversion of carbon monoxide and hydrogen to C₅⁺ hydrocabon mixtures using a system of a Fischer-Tropsch catalyst and an FCC catalyst, which system is easier to prepare.
A second object is to provide a process using a catalyst system which can be used more flexibly according to need.
A third object is to provide an Inexpensive catalyst system.

The prior art only discloses the use of spent FCC catalyst in a Fischer-Tropsch process. It is a fourth object of the present invention to enlarge the scope of FCC catalyst to be used in Fischer-Tropsch processes by using also other types of FCC catalysts. US-A-4 906 671 describes a process for producing diesel from hydrogen and carbonoxides using a catalyst system comprising a FCC catalyst and a FT catalyst.

US3254023, example 6 discusses a process in which a Fischer-Tropsch type synthesis is utilized as an exothermic addition reaction, the heat derived therefrom serving to effect an endothermic dehydration reaction. There is discussion of a dehydration of isobutanol to isobutylene catalysed by a synthetic Y-zeolite. The reactions are carried out at atmospheric pressure.

According to the invention there is provided a process as defined in claim 1.

The process according to the invention uses Fischer-Tropsch catalyst particles and fluid catalytic cracking catalyst particles.
Hence, the catalyst composition according to the present invention can be prepared by simply mixing existing Fischer Tropsch catalyst particles and FCC catalyst particles. Its preparation does not require industrially undesired impregnation steps.

In one embodiment, the Fischer-Tropsch catalyst particles and the FCC catalyst particles may be used in the form of shaped bodies in which both particles are embedded. Examples of shaped bodies are spray-dried particles (microspheres), extrudates, pellets, spheres, etc.

Such shaped bodies can be prepared by shaping a physical mixture of Fischer-Tropsch catalyst particles and FCC catalyst particles. Suitable methods to obtain such shaped bodies include spray-drying, pelletising, extrusion (optionally combined with kneading), beading, or any other conventional shaping method used in the catalyst and absorbent fields or combinations thereof.
For instance, if the preparation of the Fischer-Tropsch catalyst particles involves a spray-drying step, it is possible to add the FCC catalyst to the Fischer-Tropsch catalyst before spray-drying and subsequently spray-dry the resulting mixture.

If desired, a matrix or binding material can be added to improve the mechanical strength of the shaped bodies. Examples of suitable matrix or binding materials are alumina, silica, clays, and mixtures thereof. Matrix or binding materials comprising alumina are generally preferred. The matrix or binding material, if present, is preferably present in an amount of 10-40 wt%, more preferably 15-35 wt%, and most preferably 25-35 wt%, based on the total weight of the catalyst composition.

The term 'FCC catalyst' includes fresh FCC catalysts, spent FCC catalysts and equilibrium catalysts (E-cat). A spent FCC catalyst is less expensive than a fresh FCC catalyst. Furthermore, its use results in re-use of waste materials, which is economically and environmentally favourable.

If the FCC catalyst particles and the Fischer-Tropsch catalyst particles are not in the form of shaped bodies in which both particles are embedded, the Fischer-Tropsch catalyst particles and the FCC catalyst particles can be dosed individually - according to need - to the Fischer-Tropsch unit. This creates great flexibility. For instance, if the process conditions change during processing or if one of the catalysts deactivates faster than the other, one of the catalysts might be added with a faster dosing rate than the other.

Furthermore, the quality of E-cat or spent FCC catalyst will vary from batch to batch. This difference can be compensated for by adapting the dosing rate of the FCC catalyst particles compared to that of the Fischer-Tropsch catalyst particles.
In addition, it is possible to either use both types of catalyst particles in the second step of the Flscher-Tropsch process, or to use the Fischer-Tropsch catalyst particles in the second step and the FCC catalyst particles in the third step.

In the process according to the invention zeolite Y-containing FCC catalysts are used. Such FCC catalysts generally contain zeolite Y, clay (e.g. kaolin, metakaolin, bentonite), silica, alumina, rare-earth metal compounds, etc.
Examples of suitable metals are rare earth metals, e.g. Ce, La, and transition metals of Groups IV-VIII of the Periodic System, e.g. V, Cr, Mn, Fe, Co, Ni, Cu, Zr, Nb, Ru, Re, etc. The metal compounds can serve to, e.g., increase the particle strength (e.g. La compounds), enhance the catalyst's stability (e.g. Ni compounds), or enhance CO conversion (e.g. Fe, Co, or Ru compounds).
This metal compound is preferably present in or on the FCC catalyst particles in amounts of 0.1 to 10 wt%, more preferably 0.3 to 2 wt%, calculated as oxide, and based on the total weight of metal-containing FCC catalyst.
The metal compound can be deposited on the FCC catalyst particles in any manner known in the art. Examples of such methods are impregnation, ionexchange, and deposition precipitation of soluble metal salts.
If desired, the metal-deposited FCC catalyst particles is calcined and/or prereduced after the metal compound has been deposited.

An additional advantage of using a spent FCC catalyst compared to a fresh FCC catalyst is that a spent FCC catalyst will generally contain a desired metal compound, due to the fact that the hydrocarbon feed to be cracked in an FCC unit generally contains various metals - e.g. nickel, vanadium. Consequently, no additional deposition step is required to introduce such a metal compound.

The Fischer-Tropsch catalyst can be any conventional Fischer-Tropsch catalyst, preferably comprising iron and/or cobalt. For the preparation of such catalysts it is referred to, e.g., WO 01/97968, WO 01/89686/ and WO 01/70394.
The Fischer-Tropsch catalyst can be promoted with various metals, e.g. Al, Ti, Cr, Mn, Ca, Na and/or K. Furthermore, the Fischer-Tropsch catalyst particles can contain binder materials, such as silica and/or alumina.

Both the FCC catalyst particles and the Fischer-Tropsch catalyst particles can be used in the second step of the Fischer-Tropsch process, either in the form of separate particles, or in the form of shaped bodies in which both particles are embedded. Based on the total weight of FCC catalyst particles and Fischer-Tropsch catalyst particles, the FCC catalyst particles are preferably be used in an amount of 5 to 40 wt%, more preferably from 10 to 30 wt%.

The second step can be carried out in any suitable reactor, such as a (fixed) fluldised bed reactor. The temperature ranges preferably from 250° to 400°C, more preferably from 300° to 370°C, and most preferably from 330° to 350°C.
The pressure ranges from 10 to 60 bar, more preferably 15 to 30 bar, and most preferably about 20 bar.
The H₂/CO volume ratio preferably ranges from 0.2 to 6.0, preferably 0.5-6, most preferably 1-3.

The third step is generally conducted at temperatures of 150 to 600°C, more preferably 200 to 500°C, and most preferably 300 to 400°C The pressure preferably ranges from 5 to 60 bar, more preferably from 15 to 40 bar, and most preferably from 20 to 30 bar.

The resulting hydrocarbon product preferably contains, on a mass basis, at least 35%, more preferably at least 45%, and most preferably at least 50% of C₅⁺ compounds. The process may be used for the production of branched hydrocarbons, olefins, and/or aromatics. Preferably, the process is used for the production of liquid fuel, especially diesel and gasoline, and preferably unleaded gasoline.

### EXAMPLE

The following experiments illustrate the suitability of zeolite-Y-based FCC catalysts (fresh and E-cat), for the isomerisation of linear olefinic products under typical Fischer-Tropsch process conditions.
Catalysts which are suitable for this purpose can be used either in the second step (as co-catalyst) or in the third step of the Fischer-Tropsch process in order to enhance the isomerisation of the linear olefinic products.

To this end, the performance of the FCC catalysts was tested in a hydroisomerization of 1-hexene. The reaction conditions (temperature, total pressure and dihydrogen pressure) for the performance tests were identical to the conditions present in a typical high temperature Fischer-Tropsch process:

| | |
|---|---|
| Temperature : | 340°C |
| Total Pressure : | 20 bar |
| Catalyst intake : | 2.2 g |
| WHSV, 1-Hexene : | 2.85 g/g/hr (based on zeolite present) |
| H₂ Partial pressure : | 9 bar |
| N₂ Partial pressure : | 10.8 bar |
| 1-Hexene Partial pressure : | 0.22 bar |
| Mole ratio H₂/1-Hexene : | 40.9 |
| Mole ratio N₂/1-Hexene : | 49.1 |

The FCC catalysts were reduced in situ in the reactor under 20 bar hydrogen pressure 340°C for 1 hr. After the reduction procedure was completed, the nitrogen flow was introduced and subsequently 1-hexene was dosed (0.11 ml/min). The composition of the reaction product was followed by on-line GC analysis.

Three different types of FCC catalysts were tested according to this procedure: a fresh FCC catalyst containing a low amount of rare earth (RE), a fresh FCC catalyst containing a high amount of rare earth metals, and an equilibrium FCC catalyst (E-cat) resulting from the FCC catalyst with a low amount of RE.
The product distribution obtained in these tests at 0.5 hr and at 17.5 hr runtime are presented in Tables 1 and 2, respectively.

In these Tables, *n*-*C₆* refers to normal C₆ paraffins, *i*-*C₆* refers to branched C₆ paraffins, *n*-*C₆*= refers to normal C₆ olefins, *i*-*C₆*= refers to branched C₆ olefins, and <*C₆* and *>C₆* refers to compounds with less and more than 6 carbon atoms, respectively.

**Table 1 - test results at 0.5 hr. runtime**

| | Fresh FCC | Fresh FCC | E-cat |
|---|---|---|---|
| | low RE | high RE | |
| Conversion 1-hexene, wt% | 93.8 | 99.4 | 94.0 |
| n-C₆, wt% | 19.8 | 28.5 | 29.6 |
| i-C₆, wt% | 19.2 | 41.6 | 13.7 |
| n-C₆=, wt% | 9.4 | 0.7 | 24.3 |
| i-C₆=, wt% | 32.8 | 3.2 | 24.5 |
| <C₆, wt% | 10.9 | 20.2 | 4.4 |
| >C₆, wt% | 8.2 | 6.0 | 3.7 |
| i-C₆ + i-C₆=, wt% | 52.0 | 44.8 | 38.2 |

**Table 2 - test results at 17.5 hr. runtime**

| | Fresh FCC | Fresh FCC | E-cat |
|---|---|---|---|
| | low RE | high RE | |
| Conversion 1-hexene, wt% | 90.8 | 91.4 | 91.8 |
| n-C₆, wt% | 10.0 | 11.0 | 15.5 |
| i-C₆, wt% | 12.8 | 14.9 | 9.3 |
| n-C₆=, wt% | 20.2 | 15.1 | 39.3 |
| i-C₆=, wt% | 47.3 | 45.6 | 30.6 |
| <C₆, wt% | 3.4 | 5.3 | 3.0 |
| >C₆, wt% | 6.5 | 8.4 | 2.7 |
| i-C₆ + i-C₆=, wt% | 60.1 | 60.5 | 39.9 |

As can be seen from these tables, the fresh FCC catalyst with a low amount of RE has a high selectivity to branched C₆ olefins (i-C₆=) and branched C₆ paraffins (i-C₆). The total amounts of isomerized products at 0.5 hr and 17.5 hr runtime were 52.0 wt% and 60.1 wt%, respectively. This high isomerization selectivity was accompanied with a low level of cracking; only 3.4 wt% of products smaller than C₆ (<C₆) were obtained at 17.5 hr runtime. The amount of aromatic products was far below 1 wt% during the whole run.

The fresh FCC catalyst with a high amount of RE also showed a high selectivity to branched C₆ olefins (i-C₆=) and branched C₆ paraffins (i-C₆). The total amounts of isomerized products at 0.5 hr and 17.5 hr runtime were 44.8 wt% and 60.5 wt%, respectively. The level of cracking was 5.3 wt% at 17.5 hr runtime. The amount of aromatic products was far below 1 wt% during the whole run.

The equilibrium FCC catalyst showed a somewhat lower selectivity to branched C6 olefins (i-C6=) and branched C6 paraffins (i-C6) than the fresh FCC catalysts. The total amounts of isomerized products at 0.5 hr and 17.5 hr runtime were 38.2 wt% and 39.8 wt%, respectively. The level of cracking was only 3.0 wt% at 17.5 hr runtime. Again, the amount of aromatic products was far below 1 wt% during the whole run.
Although the level of isomerization of this E-cat was lower than that of the fresh FCC catalysts, it is still acceptable for use in the Fischer-Tropsch product, especially as co-catalyst in the second step..

These experiments show that FCC catalysts are able to isomerise linear olefinic hydrocarbons under typical Fischer-Tropsch conditions. This indicates their suitability for use in the second and third step of the Fischer-Tropsch process.

## Claims

1. Fischer-Tropsch process for the conversion of carbon monoxide and hydrogen to C₅⁺ hydrocarbon mixtures in which process use is made of Fischer-Tropsch catalyst particles and zeolite Y-containing fluid catalytic cracking catalyst particles, said process comprising contacting the carbon monoxide and hydrogen with the Fischer-Tropsch catalyst particles at a pressure in the range from 10 to 60 bar leading to hydrocarbons and water, and isomerising the hydrocarbons with the fluid catalytic cracking catalyst particles.

2. Process according to claim 1 wherein the mixture of carbon monoxide and hydrogen is contacted with a mixture of Fischer-Tropsch catalyst particles and fluid catalytic cracking catalyst particles, wherein the fluid catalytic cracking catalyst particles comprise from 5 to 40 wt% of said mixture.

3. Process according to claim 2 wherein the Fischer-Tropsch catalyst particles and the fluid catalytic cracking catalyst particles are dosed individually to the reaction mixture.

4. Process according to claim 2, wherein the Fischer-Tropsch catalyst particles and fluid catalytic cracking catalyst particles are used in the form of shaped bodies in which both particles are embedded.

5. Process according to claim 1 wherein the step of contacting Fischer Tropsch catalyst particles with a mixture of carbon monoxide and hydrogen to form a C₅₊ hydrocarbon mixture is followed by a separate step of contacting the C₅₊ hydrocarbon mixture with the fluid catalytic cracking catalyst particles.

6. Process according to any one of the preceding claims wherein the Fischer-Tropsch catalyst particles comprise iron.

7. Process according to any one of the preceding claims wherein the Fischer-Tropsch catalyst particles comprise cobalt.

8. Process according to any one of the preceding claims wherein the fluid catalytic cracking catalyst is a spent or equilibrium fluid catalytic cracking catalyst.

9. Process according to any one of the preceding claims wherein a metal compound has been deposited on the fluid catalytic cracking catalyst particles.

10. Process according to claim 1 comprising:
a first step involving reacting a source of carbon with a source of oxygen to form a mixture of carbon monoxide and hydrogen;
a second step in which the carbon monoxide and hydrogen are contacted with the Fischer-Tropsch catalyst particles leading to hydrocarbons and water; and
a third step in which the hydrocarbons formed in the second step are isomerised; wherein
the zeolite Y-containing fluid catalytic cracking catalyst particles are used in the third step.

11. Process according to any one of the proceeding claims in which the fluid catalytic cracking catalyst particles isomerise linear olefinic hydrocarbons.

## Patentansprüche

1. Fischer-Tropsch-Verfahren zur Umwandlung von Kohlenmonoxid und Wasserstoff in C₅⁺-Kohlenwasserstoffgemische, wobei in diesem Verfahren Fischer-Tropsch-Katalysatorteilchen und Zeolith-Y-haltige FCC-Katalysatorteilchen (FCC = Fluid Catalytic Cracking) verwendet werden, wobei das Verfahren das In-Kontakt-Bringen des Kohlenmonoxids und Wasserstoffs mit den Fischer-Tropsch-Katalysatorteilchen unter einem Druck im Bereich von 10 bis 60 bar, was zu Kohlenwasserstoffen und Wasser führt, und das Isomerisieren der Kohlenwasserstoffe mit den FCC-Katalysatorteilchen umfasst.

2. Verfahren gemäß Anspruch 1, wobei das Gemisch aus Kohlenmonoxid und Wasserstoff mit einem Gemisch von Fischer-Tropsch-Katalysatorteilchen und FCC-Katalysatorteilchen in Kontakt gebracht wird, wobei die FCC-Katalysatorteilchen 5 bis 40 Gew.-% des Gemischs umfassen.

3. Verfahren gemäß Anspruch 2, wobei die Fischer-Tropsch-Katalysatorteilchen und die FCC-Katalysatorteilchen dem Reaktionsgemisch getrennt zudosiert werden.

4. Verfahren gemäß Anspruch 2, wobei die Fischer-Tropsch-Katalysatorteilchen und die FCC-Katalysatorteilchen in Form von Formkörpern, in die beide Teilchen eingebettet sind, verwendet werden.

5. Verfahren gemäß Anspruch 1, wobei dem Schritt des In-Kontakt-Bringens der Fischer-Tropsch-Katalysatorteilchen mit dem Gemisch aus Kohlenmonoxid und Wasserstoff unter Bildung eines C₅⁺ -Kohlenwasserstoffgemischs ein getrennter Schritt des In-Kontakt-Bringens des C₅⁺ -Kohlenwasserstoffgemischs mit den FCC-Katalysatorteilchen folgt.

6. Verfahren gemäß einem der vorstehenden Ansprüche, wobei die Fischer-Tropsch-Katalysatorteilchen Eisen umfassen.

7. Verfahren gemäß einem der vorstehenden Ansprüche, wobei die Fischer-Tropsch-Katalysatorteilchen Cobalt umfassen.

8. Verfahren gemäß einem der vorstehenden Ansprüche, wobei der FCC-Katalysator ein verbrauchter FCC-Katalysator oder Gleichgewichts-FCC-Katalysator ist.

9. Verfahren gemäß einem der vorstehenden Ansprüche, wobei auf den FCC-Katalysatorteilchen eine Metallverbindung abgeschieden ist.

10. Verfahren gemäß Anspruch 1, umfassend:
einen ersten Schritt, der das Umsetzen einer Kohlenstoffquelle mit einer Sauerstoffquelle unter Bildung eines Gemischs aus Kohlenmonoxid und Wasserstoff beinhaltet;
einen zweiten Schritt, in dem das Kohlenmonoxid und der Wasserstoff mit den Fischer-Tropsch-Katalysatorteilchen in Kontakt gebracht werden, was zu Kohlenwasserstoffen und Wasser führt; und
einen dritten Schritt, in dem die im zweiten Schritt gebildeten Kohlenwasserstoffe isomerisiert werden; wobei
die Zeolith-Y-haltigen FCC-Katalysatorteilchen im dritten Schritt verwendet werden.

11. Verfahren gemäß einem der vorstehenden Ansprüche, wobei die FCC-Katalysatorteilchen lineare olefinische Kohlenwasserstoffe isomerisieren.

## Revendications

1. Procédé de Fischer-Tropsch pour la conversion de monoxyde de carbone et d'hydrogène en mélanges d'hydrocarbures C₅⁺ dans lequel on utilise des particules de catalyseur Fischer-Tropsch et des particules de catalyseur fluide de craquage catalytiques contenant une zéolite Y, ledit procédé comprenant la mise en contact de monoxyde de carbone et d'hydrogène avec les particules de catalyseur Fischer-Tropsch à une pression comprise entre 10 et 60 bars, de manière à obtenir des hydrocarbures et de l'eau, et l'isomérisation des hydrocarbures avec les particules de catalyseur fluide de craquage catalytique.

2. Procédé selon la revendication 1, dans lequel le mélange de monoxyde de carbone et d'hydrogène entre en contact avec un mélange de particules de catalyseur Fischer-Tropsch et de particules de catalyseur fluide de craquage catalytique dans lequel les particules de catalyseur de craquage catalytique fluides constituent de 5 à 40% en poids dudit mélange.

3. Procédé selon la revendication 2, dans lequel les particules de catalyseur Fischer-Tropsch et les particules de catalyseur de craquage catalytique fluides sont introduites individuellement dans le mélange de réaction.

4. Procédé selon la revendication 2, dans lequel les particules de catalyseur Fischer-Tropsch et les particules de catalyseur de craquage catalytique fluides sont utilisées sous la forme de corps façonnés, dans lesquels les deux types de particules sont intégrés.

5. Procédé selon la revendication 1, dans lequel l'étape consistant à mettre en contact les particules de catalyseur Fischer Tropsch avec un mélange de monoxyde de carbone et d'hydrogène, pour former un mélange d'hydrocarbures C₅₊ est suivie d'une étape séparée de mise en contact du mélange d'hydrocarbures C₅₊ avec les particules de catalyseur de craquage catalytique fluides.

6. Procédé selon l'une quelconque des revendications précédentes, dans lequel les particules de catalyseur Fischer-Tropsch comprennent du fer.

7. Procédé selon l'une quelconque des revendications précédentes dans lequel les particules de catalyseur Fischer-Tropsch comprennent du cobalt.

8. Procédé selon l'une quelconque des revendications précédentes, dans lequel le catalyseur fluide de craquage catalytique est un catalyseur fluide de craquage catalytique à l'équilibre ou usé.

9. Procédé selon l'une quelconque des revendications précédentes dans lequel un composé métallique a été déposé sur les particules de catalyseur fluide de craquage catalytique.

10. Procédé selon la revendication 1, comprenant :
une première étape impliquant la réaction d'une source de carbone avec une source d'oxygène pour former un mélange de monoxyde de carbone et d'hydrogène ;
une deuxième étape dans laquelle le monoxyde de carbone et l'hydrogène sont mis en contact avec les particules de catalyseur Fischer-Tropsch donnant des hydrocarbures et de l'eau ; et
une troisième étape dans laquelle les hydrocarbures formés dans la seconde étape sont isomérisés ; dans lequel
les particules de catalyseur fluide de craquage catalytique contenant une zéolite Y sont utilisées dans la troisième étape.

11. Procédé selon l'une quelconque des revendications précédentes, dans lequel les particules de catalyseur fluide de craquage catalytique isomérisent les hydrocarbures oléfiniques linéaires.
